

1

2,944,971

## STABLE ANTI-CORROSION LUBRICANT COMPOSITION

Milton P. Kleinholtz, Homewood, Ill., assignor to Sinclair Refining Company, New York, N.Y., a corporation of Maine

No Drawing. Filed May 3, 1956, Ser. No. 582,342

3 Claims. (Cl. 252—32.7)

This invention relates to lubricants, and more particularly to lubricating oils which contain a basic barium mahogany sulfonate in combination with the oil-soluble nickel salts of dithiophosphoric acid diesters.

In the development of lubricating oils, a great variety of additives have heretofore been suggested for use in mineral oil bases for the protection of metal surfaces, which come in contact with the base oil under conditions of severe service, particularly internal combustion engines and the like wherein oxidation of the base oil, bearing corrosion, frictional and corrosive wear, and varnish and sludge formation are frequently encountered. Many of these additives, which are known to display oxidation-inhibiting action in hydrocarbon oils, for example, the metal salts of esters of dithiophosphoric acid, have in general been used in conjunction with other additives, such as the oil-soluble organic sulfonates, to effect both stabilization and detergency characteristics in various types of mineral oil lubricating compositions.

In accordance with my invention a new mineral oil lubricating composition has been discovered wherein a particular combination of additives comprising a basic barium oil-soluble petroleum or mahogany sulfonate and the nickel salts of dithiophosphoric acid diesters is employed to lessen the oxidation of the base oil and the corrosive effects of refined lubricating oils in contact with metal surfaces. These additives in combination with a mineral lubricating oil base have been found to promote engine cleanliness and are particularly effective in reducing the corrosion of silver bearings which are employed in railroad, submarine and certain other internal combustion engines.

In carrying out the preparation of the lubricating oil compositions of this invention, a minor or small amount of oil-soluble nickel dithiophosphate is added to a suitable mineral oil base which also contains a basic barium mahogany sulfonate blended to give a barium content of about 0.2 to 2.0 percent by weight based on the total weight of the mineral oil composition. The nickel dithiophosphate is blended in a minor amount to give a final phosphorus content of about 0.03 to 0.3 percent by weight of the total composition and as shown hereinafter, this particular metal salt of the dithiophosphoric acid diester is an exceptionally good oxidation and bearing corrosion inhibitor when used in combination with the basic barium mahogany sulfonate.

The nickel dithiophosphates employed in the lubricating compositions of the present invention can be obtained from a wide variety of diester dithiophosphoric acids conventionally prepared by reacting a sulfide of phosphorus, such as phosphorus pentasulfide, with an alcohol, phenol or mercaptan. The organic groups in the acid esters may be aryl, alkyl, aralkyl or cycloalkyl groups which contain from about 4 to 20 carbon atoms, preferably about 6 to 14 carbon atoms, and may be further substituted in the organic portion. Suitable alcohols which may be employed in preparing the acid esters include oxo-alcohols, primary and secondary alcohols such

2

as 2-methylamyl alcohol, 4-methylpentanol-2, 2-methylpentanol-1, 2-ethylhexanol, di-isopropyl carbinol, cyclohexanol, butanol-1 and octadecanol-1, or mixtures of high and low molecular weight alcohols. Other hydroxyl-containing materials which can be reacted with phosphorus sulfide include phenols and alkylated phenols such as di-octylphenol, tri-isobutylphenol and the like. A particularly suitable nickel dithiophosphate which may be employed to advantage with the basic barium sulfonate is the nickel salt prepared from a di-2-ethylhexyl dithiophosphate obtained by reacting a technical mixture of 2-ethylhexanol with phosphorus pentasulfide.

The sulfonates employed in the lubricating compositions of my invention are the basic barium salts derived from the oil-soluble sulfonic acids produced in the treatment of petroleum hydrocarbons with a sulfonating agent such as sulfuric acid or sulfur trioxide. The preferentially oil-soluble sulfonic acids, generally referred to as mahogany acids, are conveniently employed as a concentrate in the oil from which they are derived and may be prepared by sulfonating a suitable petroleum distillate with fuming sulfuric acid to obtain approximately a 10 weight percent concentration of mahogany acid in the acid oil, or by sulfonating with sulfur trioxide, in which case approximately a 20% concentration can be obtained. The useful mahogany acids, which generally have a molecular weight of about 300 to 500 or higher, show a titratable acidity and may be converted into the basic barium salts by neutralization of the acid oil with an excess of basic barium compound to obtain a basic sulfonate of higher metal content than the normal salt. Generally, at least about 1.5 equivalents of the barium compound are reacted. If desired, the basic metal sulfonate can be carbonated by treatment with carbon dioxide at atmospheric or slightly elevated pressure until the strong basicity of the sulfonate is reduced from a pH of about 14 to a pH between about 7 to 8. In the practice of this invention the basic barium sulfonate can be prepared by reacting a sulfonated sweet West Texas gas oil fraction with a theoretical excess of basic barium oxide. Although the mahogany acids may, for example, contain a sulfonate concentration of about 10%, introduction of barium (3.5%) gives a barium sulfonate concentration of about 13%.

The mineral oil base stock used in the present invention is of lubricating viscosity and can be a solvent extracted or solvent refined oil obtained in accordance with conventional methods of solvent refining lubricating oils. Generally, lubricating oils have viscosities from about 35 to 250 SUS at 210° F. The base oil may be derived from paraffinic, naphthenic, asphaltic or mixed base crudes, and if desired, a blend of solvent-treated Mid-Continent neutrals and Mid-Continent bright stocks may be employed. A particularly suitable base oil used in the preparation of the compositions described hereinafter is a solvent-treated Mid-Continent neutral having a viscosity index of about 95.

The following examples, which are not to be construed as limiting the scope of the invention, are offered to illustrate further the method of preparing the novel lubricating compositions of the present invention.

### EXAMPLE I

#### Preparation of basic barium sulfonate

A 270 SUS at 100° F. viscosity Sweet West Texas gas oil fraction was treated with four 28 pound per barrel dumps of 20% oleum. The sludge was removed after each oleum dump. The acid-treated oil was freed of SO<sub>2</sub> by air blowing to leave a solution of approximately 10% mahogany sulfonic acid in oil having an acid No. of 14.1. The acid oil was neutralized by mixing it with

approximately 250% theoretical barium oxide in water solution for several hours at 160° to 180° F. followed by dehydration by raising the temperature to 300° F. The product was filtered with Supercel to obtain a basic barium sulfonate which analyzed as follows:

|                       |      |
|-----------------------|------|
| Percent barium.....   | 3.36 |
| Base No. to pH 4..... | 13.9 |

The following Examples II and III illustrate the preparation of the nickel salt of di-2-ethylhexyl dithiophosphoric acid using nickel carbonate or nickel oxide of small crystallite size.

#### EXAMPLE II

2-ethylhexanol (5200 grams) was placed in a 12 liter round bottomed, three-neck flask. A glass agitator and thermometer were fitted to the flask. The temperature of the alcohol was increased to 168° F. by heating. At this point, phosphorus pentasulfide was slowly added to the agitated mixture at a constant rate and over a period of 5 hours. The total amount of phosphorus pentasulfide used was 2220 grams. To remove traces of unreacted products in the solution the acid was filtered through paper at room temperature.

354 grams of the di-2-ethylhexyl dithiophosphoric acid thus obtained were then placed in a 1 liter three-neck flask. To the acid were added 300 grams toluene and 10 grams water. The temperature was increased to 160-200° F. and 60 g. nickel carbonate (ous) was slowly added. As the nickel carbonate was added the solution became purple in color. After about 5 hours reaction time the material was filtered through Hy-Flow filter aid and paper. To remove solvent toluene, the salt solution was stripped at a temperature of 170° F. and 10-15 mm. Hg. The yield of nickel salt formed, calculated in weight of acid used was 95%.

#### Analysis of sample

| Theory  |         | Found   |         |
|---------|---------|---------|---------|
|         | Percent |         | Percent |
| NI..... | 7.68    | NI..... | 16.41   |
| S.....  | 16.78   | S.....  | 14.60   |
| P.....  | 8.13    | P.....  | 17.24   |

Calc.-Ratio NI/S=0.457 NI/S=0.440

Calc.-Ratio P/S=0.485 P/S=0.496

<sup>1</sup> Low Ni, S, P, believed to be due to the presence of some solvent.

#### EXAMPLE III

354 grams of di-2-ethylhexyl dithiophosphoric acid as prepared in Example II were placed in a 1 liter three-neck flask. To the acid were added 200 grams toluene and 7 grams water. The temperature of the mixture was increased to 160° F. At this point, 40 grams of NiO were added.

The oxide used was 71% nickel and it had 40 to 60 A. crystallite size (as determined by X-ray methods). After about 7 hours at 160-170° F., the dark purple solution was filtered through Hy-Flow filter aid and paper. The toluene was removed from the filtered solution by stripping to a pot temperature of 170° F. and 10-15 mm. Hg pressure. The yield of nickel salt formed, calculated on weight of acid used, was 92%.

#### Analysis of Sample

| Theory  |         | Found   |         |
|---------|---------|---------|---------|
|         | Percent |         | Percent |
| NI..... | 7.68    | NI..... | 7.68    |
| S.....  | 16.78   | S.....  | 16.20   |
| P.....  | 8.13    | P.....  | 8.02    |

Sp. Gr. 60/60=1.0781

#### EXAMPLE IV

The following Table I lists the analyses of fourteen different metal salts of di-2-ethylhexyl dithiophosphoric acid.

TABLE I  
Analysis of metal di-2-ethylhexyl dithiophosphates

| Metal                               | Percent Metal |        | Percent P |        | Percent S |        |
|-------------------------------------|---------------|--------|-----------|--------|-----------|--------|
|                                     | Found         | Theory | Found     | Theory | Found     | Theory |
| <b>Nickel:</b>                      |               |        |           |        |           |        |
| A Made from NiO.....                | 7.68          | 7.68   | 8.02      | 8.13   | 16.20     | 16.78  |
| B Made from NiCO <sub>3</sub> ..... | 6.41          | -----  | 7.24      | -----  | 14.60     | -----  |
| Zinc.....                           | 7.99          | 8.44   | 8.42      | 8.04   | 16.20     | 16.60  |
| Barium.....                         | 16.31         | 16.30  | 7.58      | 7.35   | 15.10     | 15.20  |
| Calcium.....                        | 5.86          | 5.38   | 8.37      | 8.30   | 16.4      | 17.15  |
| Magnesium.....                      | 3.16          | 3.33   | 8.46      | 8.50   | 16.93     | 17.55  |
| Cadmium.....                        | 13.70         | 13.72  | 7.56      | 7.58   | 15.10     | 15.62  |
| Lithium.....                        | 1.84          | 1.93   | 8.61      | 8.62   | 17.18     | 17.81  |
| Sodium.....                         | 6.05          | 6.12   | 8.22      | 8.25   | 16.80     | 17.0   |
| Potassium.....                      | 8.68          | 9.98   | 7.96      | 7.91   | 15.20     | 16.31  |
| Copper.....                         | 9.00          | 8.28   | 7.91      | 8.08   | 14.10     | 16.65  |
| Tin.....                            | 14.24         | 14.40  | 7.40      | 7.54   | 15.15     | 15.55  |
| Lead.....                           | 21.2          | 22.7   | 6.78      | 6.79   | 14.4      | 14.0   |
| Iron.....                           | 6.85          | 7.34   | 8.19      | 8.15   | 16.60     | 16.80  |
| Cobalt.....                         | 7.52          | 7.71   | 8.10      | 8.14   | 16.60     | 16.78  |

#### EXAMPLE V

The following Table II lists the results of laboratory oxidation tests run on oil blends including 27% of basic barium mahogany sulfonate concentrate containing about 13% sulfonate prepared essentially as in Example I. Each of the fourteen metal dithiophosphates shown in Table I were blended to a common phosphorus level of 0.094% in a 95 V.I. 160 SUS vis/100° F. Mid-Continent neutral base. The oxidation test consisted of bubbling 5 liters of oxygen per hour through 300 grams of oil blend at 285° F. in the presence of a copper-lead catalyst for 144 hours for analysis. 60 gram samples of oil were taken at 48, 96 and 144 hours. After each sampling except the last, 60 grams of fresh oil were added as make-up. The results shown in Table II below are from the 144 hour samples. Except where indicated, all the metal salts were obtained from the di-2-ethylhexyl dithiophosphates prepared essentially as in Example II.

It will readily be seen from the results of the severe oxidation test in Table II that the additive combination of the present invention easily gave the best results. The nickel salts of dithiophosphoric acid diesters formed the least sludge or varnish, contained the least pentane insolubles, gave the least viscosity rise and effected the lowest copper-lead catalyst loss. As also shown, the nickel dithiophosphate prepared from nickel carbonate performed better than that prepared from nickel oxide.

#### EXAMPLE VI

The silver corrosion inhibiting properties of the lubricating oil composition prepared from the additives described in Examples II and III and the basic barium sulfonate and base oil of Example V were determined by stirring a sample of oil for 72 hours in the presence of silver and copper test specimens, after which the silver specimen was cleaned with a KCN solution and its weight change determined. This test was run at both 285° F. and 325° F. although the former temperature is most commonly used.

In this test, the oil blends containing the nickel di-2-ethylhexyl dithiophosphate allowed the lowest loss in weight of the silver at 285° F., and gave good results at 325° F. This indicates that these oils, adjusted in viscosity, have less tendency to corrode silver bearings, such as those commonly found in railroad, submarine and certain other internal combustion engines, whereas many of the other oils tested would prove too corrosive. Except as indicated, all the metal salts were prepared from

TABLE II  
Oxidation tests

| Metal Dithiophosphates              | Viscosity Rise at 100° F., SUS | Percent Pentane Insolubles | Acid Number | Loss in Cu-Pb Catalyst Wt., Mgs. | Appearance of Tube               |
|-------------------------------------|--------------------------------|----------------------------|-------------|----------------------------------|----------------------------------|
| Nickel:                             |                                |                            |             |                                  |                                  |
| A Made from NiO.....                | 23.7                           | 0.251                      | 5.93        | 23.3                             | Slight Sludge and Varnish.       |
| B Made from NiCO <sub>3</sub> ..... | 7.6                            | 0.016                      | 1.69        | 28.2                             | No Sludge or Varnish.            |
| Nickel <sup>1</sup> .....           | 13.2                           | 0.013                      | 3.54        | 0.2                              | Do.                              |
| Zinc.....                           | 3.6                            | 0.050                      | 1.32        | 0.3                              | Slight Sludge and Varnish.       |
| Zinc.....                           | 127.2                          | 4.922                      | 7.43        | 688.4                            | Heavy Sludge and Varnish.        |
| Barium.....                         | 114.4                          | 7.501                      | 13.02       | 297.0                            | Do.                              |
| Calcium.....                        | 150.8                          | 8.681                      | 16.23       | 447.9                            | Do.                              |
| Magnesium.....                      | 142.1                          | 6.044                      | 17.13       | 285.7                            | Do.                              |
| Cadmium.....                        | 57.7                           | 4.394                      | 7.94        | 157.3                            | Do.                              |
| Lithium.....                        | 199.2                          | 4.868                      | 15.85       | 458.7                            | Do.                              |
| Sodium.....                         | 98.1                           | 8.485                      | 15.29       | 702.5                            | Do.                              |
| Potassium.....                      | 130.1                          | 9.415                      | 17.28       | 571                              | Do.                              |
| Copper.....                         | 38.5                           | 5.28                       | 5.28        | 65.1                             | Medium Heavy Sludge and Varnish. |
| Tin.....                            | 53.1                           | 0.702                      | 2.33        | 238.8                            | Do.                              |
| Lead.....                           | 50.5                           | 3.709                      | 5.06        | 73.2                             | Do.                              |
| Iron.....                           | 46.4                           | 10.953                     | 15.07       | 467.0                            | Heavy Sludge and Varnish.        |
| Cobalt.....                         | 38.6                           | 6.22                       | 8.80        | 121.2                            | Medium Heavy Sludge and Varnish. |

<sup>1</sup> Nickel di-methylamyl dithiophosphate, made from methylamyl alcohol or 4-methylpentanol-2.<sup>2</sup> Nickel di-tertiary octylphenyl dithiophosphate.

the di-2-ethylhexyl dithiophosphate prepared essentially as in Example II.

TABLE III

| Metal Dithiophosphates              | Loss in Wt. of Silver Strip, Mgs. |              |
|-------------------------------------|-----------------------------------|--------------|
|                                     | 285° F. Test                      | 325° F. Test |
| Nickel:                             |                                   |              |
| A Made from NiO.....                | 1.6                               | 12.0         |
| B Made from NiCO <sub>3</sub> ..... | 1.7                               | 2.6          |
| Zinc.....                           | 11.6                              | 15.0         |
| Barium.....                         | 17.8                              | 54.5         |
| Calcium.....                        | 27.7                              | 37.6         |
| Magnesium.....                      | 4.5                               | 7.1          |
| Cadmium.....                        | 18.9                              | 26.0         |
| Lithium.....                        | 37.8                              | 31.1         |
| Sodium.....                         | 51.3                              | 39.9         |
| Potassium.....                      | 24.4                              | 30.4         |
| Copper.....                         | 5.5                               | 4.0          |
| Tin.....                            | 71.3                              | -----        |
| Lead.....                           | 16.4                              | 31.5         |
| Iron.....                           | 239.7                             | 177.8        |
| Cobalt.....                         | 13.9                              | -----        |
| Nickel <sup>1</sup> .....           | 10.7                              | 18.0         |
| Nickel <sup>2</sup> .....           | 0.9                               | -----        |

<sup>1</sup> Derived from methylamyl alcohol.<sup>2</sup> Derived from tertiary octyl phenol.

## EXAMPLE VII

A 36-hour L-4 Chevrolet engine test was also used in evaluating the lubricating composition prepared in accordance with this invention. In this test the engine is a conventional Chevrolet engine with 216.5 cu. in. piston displacement and a compression ratio of 6.5 to 1. The engine is operated at 3150 r.p.m. with a load of 30 B.H.P. and at a temperature at the jacket outlet of 200° F. The L-4 Chevrolet test was carried out on an SAE 10W oil containing 27% basic barium mahogany sulfonate concentrate containing about 13% sulfonate prepared essentially as in Example I, nickel di-2-ethylhexyl dithiophosphate in an amount to provide 0.075% P to the total composition, 1.4% V.I. improver and 0.005% foam inhibitor, in a 95 V.I. Mid-Continent neutral base. The oil sump temperature was maintained at 265° F. The following results were obtained.

## L-4 engine test

Varnish deposits piston skirts..... 9.5  
Total varnish and sludge..... 95  
Copper-lead bearing loss/whole bearing..... 38

Results of rocker arm shaft wear tests on oils containing a few different metal dithiophosphates and basic barium mahogany sulfonate are shown in Table IV. These 100 hour tests were run in a popular make 1955 V-8 engine which is experiencing excessive wear of this portion of the valve train in the field. A smooth contact area on the rocker arm shaft with little or no wear, is highly desirable in this test. A rough wear area accelerates the amount of wear with further running.

As readily seen in Table IV, the results of these tests show that the oils containing the nickel dithiophosphate and the basic sulfonate gave the smoothest contact areas, about 10 microinches, of the dithiophosphates tested, with very little or no wear. The original shafts show 15-25 microinches finish, indicating that the oils containing the nickel dithiophosphate have a mild, polishing action in these areas. The oils containing the other dithiophosphates and the basic sulfonate are unsatisfactory in giving coarse to rough wear areas. The rocker arm shaft wear tests were run on an SAE 10W grade oil containing 27% basic barium mahogany sulfonate concentrate comprising about 13% sulfonate, prepared essentially as in Example I, 1.4% V.I. improver, and various metal dialkyl dithiophosphates blended to a common phosphorus level of 0.12%. In tests 5 to 7 the various runs were carried out on the same reference oil except that 1.25% of sulfurized sperm oil was added as an anti-wear agent. Similarly, the lubricating compositions of this invention may contain other lubricating oil additive agents such as detergents, dyes, pour depressors, viscosity index improvers, defoamers and the like, which are designed to impart desired characteristics to the mineral oil.

TABLE IV  
Rocker arm shaft wear tests

| 65 | Metal Dithiophosphates            | Wear, Inches | Max. Surface Roughness, Micro-inches | Appearance of Contacted Shaft Area |
|----|-----------------------------------|--------------|--------------------------------------|------------------------------------|
| 70 | 1. Magnesium di-2-ethylhexyl..... | 0.0001       | 30                                   | Rather Coarse.                     |
|    | 2. Nickel di-2-ethylhexyl.....    | 0.0000       | 10                                   | Smooth and polished.               |
|    | 3. Commercial Zinc dialkyl.....   | 0.0003       | 38                                   | Coarse.                            |
|    | 4. Nickel di-methylamyl.....      | 0.0001       | 5                                    | Smooth.                            |
|    | 5. Zinc di-secondary butyl.....   | 0.0003       | 65                                   | Rough.                             |
|    | 6. Zinc di-isobutyl.....          | 0.0006       | 65                                   | Rough.                             |
| 75 | 7. Nickel di-2-ethylhexyl.....    | 0.0001       | 10                                   | Smooth.                            |

I claim:

1. A lubricating oil composition consisting essentially of a major proportion of mineral lubricating oil and minor amounts of an oil-soluble nickel dithiophosphate diester in which each organic group contains from about 4 to 14 carbon atoms, and a basic barium mahogany sulfonate formed by neutralizing a mahogany sulfonic acid with at least about 1.5 equivalents of a basic barium compound and wherein the barium content is from about 0.2 to 2.0 percent by weight and the phosphorus content is from about 0.03 to 0.3 percent by weight based on the total weight of said composition.

2. The composition of claim 1 wherein the mineral oil is a solvent-treated Mid-Continent oil.

3. The composition of claim 1 wherein said dithiophosphate is nickel di-2-ethylhexyl dithiophosphate.

References Cited in the file of this patent

UNITED STATES PATENTS

|           |               |               |
|-----------|---------------|---------------|
| 2,289,795 | McNab         | July 14, 1942 |
| 2,344,392 | Cook          | Mar. 14, 1944 |
| 2,369,632 | Cook          | Feb. 13, 1945 |
| 2,606,872 | Gasser et al. | Aug. 12, 1952 |
| 2,623,016 | Mertes        | Dec. 23, 1952 |
| 2,662,055 | Towne         | Dec. 8, 1953  |
| 2,723,234 | Asseff et al. | Nov. 8, 1955  |

FOREIGN PATENTS

|         |               |               |
|---------|---------------|---------------|
| 696,064 | Great Britain | Aug. 26, 1953 |
|---------|---------------|---------------|